

## UNITED STATES PATENT OFFICE

2,058,788

## LUBRICATING COMPOUND

Waldersee B. Hendrey, Beacon, N. Y., assignor to  
The Texas Company, New York, N. Y., a corporation of Delaware

No Drawing. Application July 10, 1933,  
Serial No. 679,717

4 Claims. (Cl. 87—9)

This invention relates to soluble oils or oil-containing compounds capable of ready dispersion in water with slight agitation whereby a stable emulsion is formed.

- 5 In the preparation of the usual soluble oils, an oil which may be of animal, vegetable or petroleum origin is combined with a soap which is both oil and water soluble. Other materials such as alcohol and excess fatty acid are usually added 10 chiefly to keep the soap and oil from separating. When this mixture is added to water, an oil-in-water emulsion forms, the soap acting as an emulsifying agent. It has been found that when emulsions of this type are used as coolants in the cutting or shaping of metals, the conditions to which 15 the emulsions are subjected often bring about the separation of the oil from its emulsified form. Furthermore, gummy compounds may be formed by the oxidation of the soaps.
- 20 I have discovered that a highly satisfactory soluble oil, which is stable under all normal conditions of use and which does not precipitate gummy compounds, may be prepared from a petroleum hydrocarbon lubricating oil in which 25 there has been dissolved an oil- and water-soluble soap and a small quantity of pine oil. When a soluble oil prepared in this manner is mixed with water, a cutting oil emulsion of extremely high stability results.
- 30 In preparing soluble oils of the type disclosed above, any one of the well-known alkali metal soaps may be used as an emulsifying agent. These include the soaps of fatty acids, rosin acids, sulfonic acids, as well as naphthenic acids 35 recoverable from petroleum. The sodium naphthenates are particularly valuable in that they are extremely stable and in that they do not affect deleteriously the metals with which they come in contact in use.
- 40 Although pine oil has been found to be a most satisfactory stabilizing agent, oxygenated terpene derivatives such as terpineol, borneol, fenchyl alcohol and camphor or mixtures of the same may be employed.
- 45 I have also discovered that the presence of a small quantity of water is desirable in the soluble oil base in that it greatly enhances the emulsification of the base with water in forming the cutting oil emulsion. The most desirable quantity of water for this purpose has been found to

be in the neighborhood of 2% but smaller or larger percentages than this may be found advantageous in particular cases.

As an example of the application of my invention, I give herewith a typical composition which, when mixed with from 5-50 parts of water, yields a cutting oil emulsion of extremely high stability:

|                                                                     | Per cent |
|---------------------------------------------------------------------|----------|
| Lubricating oil having a viscosity of 100 seconds Saybolt universal | 10       |
| Sodium naphthenate                                                  | 80       |
| Water                                                               | 16       |
| Pine oil                                                            | 2        |
|                                                                     | 2        |

In compounding this mixture, an advantageous 15 method consists in dissolving the proper proportion of naphthenic acids in about an equal amount of the petroleum hydrocarbon oil, warming the mixture and then saponifying the naphthenic acids with the proper amount of a caustic soda 20 solution. The mixture is then boiled under carefully controlled conditions to bring about the vaporization of the water. When the mixture is reduced to the proper water content, the proper proportion of pine oil and the remainder of the 25 mineral oil is added and dissolved in the mixture with stirring.

Petroleum hydrocarbon oils of widely varying characteristics may be found suitable in preparing 30 soluble oils in accordance with the present invention. The proper choice of the particular oil is dictated at all times by the use to which the final cutting oil emulsion is to be subjected. In some cases, instead of using a particular hydrocarbon oil fraction, it may be found advantageous 35 to use a mixture of petroleum hydrocarbons, which mixture may consist of a heavy lubricating oil cut back or diluted with lighter hydrocarbons.

Obviously many modifications and variations 40 of the invention, as hereinbefore set forth, may be made without departing from the spirit and scope thereof, and therefore only such limitations should be imposed as are indicated in the appended claims.

I claim:

1. A soluble oil consisting essentially of a mixture of a low viscosity mineral lubricating oil, sodium naphthenate, from 1-5% of pine oil, and about 2% of water.

2. A soluble oil consisting of from 78-82% of a light mineral lubricating oil, from 14-18% of sodium naphthenate, 2% of pine oil, and 2% of water.
- 5 3. A soluble oil consisting essentially of a mixture of mineral lubricating oil, an alkali metal soap, from 1-5% of pine oil and about 2% of water.

4. A soluble oil consisting essentially of a mixture of mineral lubricating oil, an alkali metal soap, from 1-5% of oxygenated terpene selected from the group consisting of pine oil, terpineol, borneol, fenchyl alcohol and camphor, and about 2% of water.

WALDERSEE B. HENDREY.